

## UNITED STATES PATENT OFFICE

2,405,278

## FERROALLOY BRIQUETTE AND MANUFACTURE OF SAME

Calbert L. Vance, Zanesville, Ohio, assignor to  
Ohio Ferro-Alloys Corporation, Canton, Ohio, a  
corporation of Ohio

No Drawing. Application December 11, 1943,  
Serial No. 513,953

7 Claims. (Cl. 75—44)

1

The invention relates to briquettes of metals or ferro alloys for use as additions, deoxidizers, and the like, in the making of iron and steel, as well as to the manufacture of such briquettes.

It is customary in the manufacture of iron and steel to make additions of various metals or ferro alloys such as chromium, silicon, manganese, phosphorus, and the like, to the charge or melt, either as alloys or deoxidizers.

In order to produce the desired results it is necessary that a definite quantity of the desired metal product or ferro alloy be added to the charge or melt and it is therefore necessary that each piece or lump of the metal or ferro alloy addition will have a definite metallic content.

To this end it has long been common practice to form briquettes of a definite known weight of the desired metal or ferro alloy, in finely divided form, mixed with a binder such as Portland cement, clay, lime or similar material.

The use of pitch, tar, or a mixture thereof, as a binder in the production of briquettes of various materials is not new, but to the best of my knowledge neither of these materials has ever been actually used as a binder for briquettes of metals or ferro alloys that are subjected to temperatures higher than the melting or fusion point of the pitch or tar, and it has been generally believed by the steel industry that pitch or tar do not form suitable binding agents for such use because of the erroneous belief that they would immediately burn away in the furnace permitting the briquettes to disintegrate and exposing the readily oxidizable alloys to the oxidizing flames of the furnace so that they are lost in whole or at least in part.

As an example of the erroneous belief that pitch or tar is not a suitable binder for ferro alloy briquettes attention is called to Greiner Patent No. 1,551,554 of September 1, 1925, for a Process for smelting iron alloys.

Pitch or tar were not regarded as suitable materials for binding ferro-alloy briquettes as it was believed that they would immediately burn away in the furnace and thus would not protect the alloys against the hot air in the furnace.

I have found by actual experience however that such theories were erroneous and that pitch or tar is not only a suitable binding agent but that briquettes of a mixture of ferro-alloy fragments and pitch or tar, formed under sufficient pressure, give very satisfactory results.

It is therefore the object of the present invention to provide a briquette for furnace additions composed of one or more ferro alloys in finely divided condition bound together by pitch or tar or a mixture thereof.

2

Another object is the formation of a briquette of such metalliferous products bound together with pitch or tar under extreme pressure.

A still further object is to provide a method of producing a briquette of this character by mixing ferro alloy material with a small amount of hot pitch or tar and subjecting the same to a suitable pressure to form a briquette.

Still another object of the invention is the provision of a ferro-alloy briquette for use as a furnace addition, which comprises ferro-alloy fragments bound together into a briquette with a binder of tar or pitch which is reinforced by small paper strips, leather shavings or the like, so that the briquette may withstand rough handling at low temperatures.

The above objects, together with others apparent to those skilled in the art, or which may be later referred to, may be attained by carrying out the invention in the manner hereinafter described in detail.

In carrying out the invention to produce the briquettes from any desired ferro alloy such as silicon, manganese, chromium, phosphorus, or the like, the desired alloy or alloys may be in small pieces, or in finely divided condition, or a mixture of the two. To this I add a small amount, usually about 3 to 5 per cent by weight of pitch or tar or a mixture of the two, preferably having a high melting point, and preferably hot.

The ferro alloy and binder are intermixed and may be placed in a mold of suitable size and shape to produce the briquette desired and subjected to extreme pressure, preferably about two tons per square inch or the briquette may be formed in an extruding press with less pressure.

Briquettes made in this manner have sufficient strength to withstand severe abuse at normal, and at even higher, handling and transportation temperatures. However, at temperatures well below freezing such briquettes may lose a portion of their strength.

Therefore, in cases where severe abuse is called for at low temperatures the briquettes can be reinforced by incorporating small strips of heavy paper such as wrapping paper, leather shavings, or the like, during the binding or briquette forming stage. These strips of paper or leather act like reinforcing rods in a concrete structure and sufficiently strengthen the briquettes to permit rough handling of the same at temperatures well below freezing.

Actual commercial tests of the ferro alloy briquettes described herein were made under varying conditions to determine the silicon recovery as compared to the silicon recovery from standard silvery iron. These tests are as follows:

## EXAMPLE NO. 1

Cupola 72"; using 17-ounce pressure; operation eight hours with a continuous stream of metal from the cupola. The test covers three days' operation and on the second day ferro-silicon briquettes were substituted for silvery iron on the basis of contained silicon.

## Regular charge

|                                        |               |
|----------------------------------------|---------------|
| 100 lbs. Pig iron 2.55% Si.....        | 2.50 lbs. Si  |
| 150 lbs. Return scrap 1.60% Si.....    | 2.40 lbs. Si  |
| 735 lbs. Purchased scrap 1.70% Si..... | 12.50 lbs. Si |
| 15 lbs. Silvery iron 15.75% Si.....    | 2.36 lbs. Si  |
| 1,000 lbs.                             | 19.81 lbs. Si |
|                                        | 1.98% Si      |
| 1,000.5 lbs.                           | 20.17 lbs. Si |
|                                        | 2.01% Si      |

## Briquette charge

|                                        |               |
|----------------------------------------|---------------|
| 100 lbs. Pig iron 2.55% Si.....        | 2.55 lbs. Si  |
| 150 lbs. Return scrap 1.60% Si.....    | 2.40 lbs. Si  |
| 745 lbs. Purchased scrap 1.70% Si..... | 12.67 lbs. Si |
| 5.5 lbs. Briquettes 46.5% Si.....      | 2.55 lbs. Si  |
| 1,000.5 lbs.                           | 20.17 lbs. Si |
|                                        | 2.01% Si      |

## Per cent silicon in ladle metal

| Time of test | Regular charge | Briquette charge | Regular charge |
|--------------|----------------|------------------|----------------|
| 7:00 a.m.    | 1.80           | 1.88             | 1.83           |
| 9:00 a.m.    | 1.76           | 1.81             | 1.74           |
| 11:00 a.m.   | 1.70           | 1.70             | 1.82           |
| 1:00 p.m.    | 1.83           | 1.81             | 1.86           |
| 3:00 p.m.    | 1.83           | 1.80             | 1.98           |

## EXAMPLE NO. 2

Cupola melting 16 tons per hour made four test runs as follows: Tests "A" and "C" with silvery iron and "B" and "D" replacing silvery iron with ferro-silicon briquettes as described above. Two types of iron were made each day and the charges used were as follows:

| Silvery iron            | Soft iron mix, lbs. | Pounds Si | Regular mix, lbs. | Pounds Si |
|-------------------------|---------------------|-----------|-------------------|-----------|
| Bessemer pig (Si 2.45%) | 1,025               | 25.10     | 1,025             | 25.10     |
| Returns (Si 2.10%)      | 1,320               | 27.70     | 970               | 20.40     |
| Steel scrap (Si 0.15%)  | 75                  | 0.10      | 425               | 0.63      |
| Silvery pig (Si 10.47%) | 80                  | 8.38      | 80                | 8.38      |
| Total                   | 2,500               | 61.28     | 2,500             | 54.51     |

| Silicon briquettes          | Soft iron mix, lbs. | Pounds Si | Regular mix, lbs. | Pounds Si |
|-----------------------------|---------------------|-----------|-------------------|-----------|
| Bessemer pig (Si 2.45%)     | 1,025               | 25.10     | 1,025             | 25.10     |
| Returns (Si 2.10%)          | 1,392               | 29.20     | 1,042             | 21.90     |
| Steel scrap (Si 0.15%)      | 75                  | 0.11      | 425               | 0.63      |
| Silicon (in briquette form) | 8                   | 8.00      | 8                 | 8.00      |
| Total                       | 2,500               | 62.41     | 2,500             | 55.63     |

## Analysis of heats

|                   | Test      |           |           |           |           |           |           |           |
|-------------------|-----------|-----------|-----------|-----------|-----------|-----------|-----------|-----------|
|                   | A         |           | B         |           | C         |           | D         |           |
|                   | Sample #1 | Sample #2 | Sample #1 | Sample #2 | Sample #1 | Sample #2 | Sample #1 | Sample #2 |
| Silicon, per cent | 2.32      | 1.71      | 2.32      | 1.88      | 2.31      | 1.90      | 2.37      | 2.02      |
| Total carbon      | 3.60      | 3.33      | 3.55      | 3.39      | 3.56      | 3.41      | 3.65      | 3.55      |
| Tensile, p. s. i. | 22,930    | 36,090    | 25,950    | 29,770    | 23,380    | 29,800    | 17,550    | 29,850    |
| Transverse        | 3,500     | 4,300     | 3,480     | 4,090     | 3,920     | 4,670     | 2,920     | 4,270     |
| Deflection (in.)  | .188      | .183      | .190      | .183      | .192      | .200      | .172      | .179      |
| Brinnel           | 149       | 197       | 163       | 179       | 156       | 179       | 137       | 187       |

## EXAMPLE NO. 3

|                                                                               |                  |                        |
|-------------------------------------------------------------------------------|------------------|------------------------|
| Cupola 48"; blast pressure 9 ounces<br>2.8 lbs. Si added per ton in the ladle | .12%             | .12%                   |
| 1,050 lbs. Steel scrap 14% Si.....                                            | 1.47 lbs. Si     |                        |
| 95 lbs. Silvery iron 15.75% Si.....                                           | 14.96 lbs. Si    |                        |
| 40 lbs. Spiegel iron 1.23% Si.....                                            | .49 lb. Si       |                        |
| 315 lbs. Return scrap 1.50% Si.....                                           | 4.73 lbs. Si     |                        |
| 10                                                                            | 1,500 lbs. Total | 21.65 lbs. Si 1.45% Si |
|                                                                               |                  | 1.57% Si               |

## Briquette iron charge

|                                        |                  |                        |
|----------------------------------------|------------------|------------------------|
| 1,050 lbs. Steel scrap 0.14% Si.....   | 1.47 lbs. Si     |                        |
| 30 lbs. Briquettes (OFA) 46.5% Si..... | 13.95 lbs. Si    |                        |
| 40 lbs. Spiegel iron 1.23% Si.....     | .49 lb. Si       |                        |
| 380 lbs. Return scrap 1.50% Si.....    | 5.70 lbs. Si     |                        |
| 15                                     | 1,500 lbs. Total | 21.61 lbs. Si 1.40% Si |
|                                        |                  | 1.52% Si               |

| Test No. | Si charge       | No. charges | Analysis |      |      |      |     |
|----------|-----------------|-------------|----------|------|------|------|-----|
|          |                 |             | C        | Si   | S    | P    | Mn  |
| A        | Silvery.....    | 22          | 3.17     | 1.50 |      |      | .84 |
| B        | Briquettes..... | 19          | 3.11     | 1.54 | .070 | .108 | .84 |
| C        | Silvery.....    | 20          | 3.05     | 1.51 | .074 | .099 | .89 |
| D        | Briquettes..... | 22          | 3.08     | 1.49 | .068 | .096 | .82 |

| Test No. | Tensile, p. s. i. | Transverse | Deflection |       |      |
|----------|-------------------|------------|------------|-------|------|
|          |                   |            |            | A     | .322 |
| B        | 52,120            |            |            | 3,015 | .330 |
| C        | 44,000            |            |            | 2,835 | .279 |
| D        | 50,890            |            |            | 3,605 | .391 |

The above tests prove that recovery of silicon from the product made according to this invention successfully meet the requirements for a ferro-alloy briquette for use in the cupola.

In actual use when ferro alloy briquettes made in the manner described are charged into a cupola, or into a bath of molten metal in a furnace or ladle, in either an oxidizing or reducing flame, some burning of volatile gases will be noted but the pitch or tar binder does not burn off permitting the briquettes to disintegrate, but cokes and continues to hold the briquette together protecting the readily oxidizable alloys until they are melted, alloyed, combined or used as desired.

I claim:

1. The method of making a briquette for iron or steel making additions which consists in mixing ferro-alloy fragments with a binder taken from a group consisting of tar and pitch incorporating small strips of reinforcing material into the mixture and forming the mixture into a briquette.
2. The method of making a briquette for iron or steel making additions which consists in mixing ferro-alloy fragments with a binder taken

from a group consisting of tar and pitch incorporating small strips of paper into the mixture, and forming the mixture into a briquette.

3. The method of making a briquette for iron or steel making additions which consists in mixing ferro-alloy fragments with a binder taken from a group consisting of tar and pitch incorporating leather shavings into the mixture and forming the mixture into a briquette.

4. The method of making a briquette for iron or steel making additions which consists in mixing ferro-alloy fragments with a binder of hot, high melting point pitch incorporating small strips of reinforcing material into the mixture and applying suitable pressure to form the mixture into a briquette.

10

15

5. A briquette for iron or steel making additions composed of ferro-alloy fragments and a binder taken from a group consisting of tar and pitch and small strips of reinforcing material incorporated in the briquette.

6. A briquette for iron or steel making additions composed of ferro-alloy fragments and a binder taken from a group consisting of tar and pitch and small strips of paper incorporated in the briquette.

7. A briquette for iron or steel making additions composed of ferro-alloy fragments and a binder taken from a group consisting of tar and pitch and leather shavings incorporated in the briquette.

CALBERT L. VANCE.